

E. E. SLICK.

METHOD OF FORMING FLANGED METAL WHEELS.

APPLICATION FILED NOV. 6, 1909.

965,039.

Patented July 19, 1910.

3 SHEETS—SHEET 1.

*Fig. 1.*



*Fig. 2.*



*Fig. 3.*



*Fig. 4.*



*Fig. 5.*



WITNESSES

R. A. Balderson  
Walter Tamariss

INVENTOR

E. E. Slick,  
by Baker, Rymer, Parmenter,  
his Atts.

965,039.

E. E. SLICK.  
METHOD OF FORMING FLANGED METAL WHEELS.  
APPLICATION FILED NOV. 6, 1909.

Patented July 19, 1910.

3 SHEETS—SHEET 2.

Fig. 6.



Fig. 7.



Fig. 8.



WITNESSES

R. A. Balderson  
Walter Farnam

INVENTOR  
E. E. Slick  
by Bakewell, Beynon & Parry,  
his Atts.

E. E. SLICK.

METHOD OF FORMING FLANGED METAL WHEELS.

APPLICATION FILED NOV. 6, 1909.

965,039.

Patented July 19, 1910.

3 SHEETS—SHEET 3.

Fig. 9.



Fig. 10.



Fig. 11.



WITNESSES

R. A. Balderson  
Walter Farnsworth

INVENTOR

E. E. Slick  
by Bachelor, Lawyer & Partner,  
his Atts.

# UNITED STATES PATENT OFFICE.

EDWIN E. SLICK, OF PITTSBURG, PENNSYLVANIA.

## METHOD OF FORMING FLANGED METAL WHEELS.

965,039.

Specification of Letters Patent.

Patented July 19, 1910.

Application filed November 6, 1909. Serial No. 526,533.

To all whom it may concern:

Be it known that I, EDWIN E. SLICK, of the city of Pittsburgh, county of Allegheny, and State of Pennsylvania, have invented a new and useful Method of Forming Flanged Metal Wheels, of which the following is a full, clear, and exact description, reference being had to the accompanying drawings, forming part of this specification, in which—

10 Figure 1 is a plan view of an ingot cast in accordance with my invention. Fig. 2 is a similar view showing the ingot of Fig. 1 as reduced in cross section in the first step of my improved method. Fig. 3 is a plan view showing the way in which the ingot of Figs. 1 and 2 is successively cut into wheel blanks in the next step of the method forming my invention. Figs. 4, 5, 6, 7 and 8 are sectional views showing one form of 20 reciprocating forging dies adapted to form the wheel blanks of Fig. 2 into flanged car wheels in accordance with my invention. Figs. 9, 10 and 11 are sectional views showing one form of rotary forging dies, constructed and arranged to form wheels from the blanks of Fig. 3 in accordance with my improved method.

The dies illustrated in Figs. 4, 5, 6, 7 and 8 are adapted for use with any of the well known types of reciprocating forging presses, and the dies of Figs. 9, 10 and 11 are adapted for use in connection with wheel forming apparatus constructed as shown in my Patent No. 915,232 for method of and apparatus for forging metal, dated March 16, 1909, or my co-pending application for manufacture of wheels, Serial No. 380,678, filed June 25, 1907.

This invention relates to the manufacture 40 of forged metal wheels having hub and rim portions joined by a continuous web portion and it more particularly relates to wheels formed integral and having a web, a hub and a flanged tread or rim portion.

45 The object of the invention is to provide a novel method of forming such wheels in a series of related steps starting with the casting operation and ending with the forged wheel, by the use of which, strong, durable 50 wheels are obtained in which the surface of the entire flange and tread portions of the wheel is formed of the surface of the cut side of the blank and the flanges and tread portions are formed of metal displaced from between the axial center and the periphery of the cast blank.

A further object of the invention is to provide an improved method of making wheels in which the fiber of the metal of the wheel is disposed in the same direction relative to the axis of the wheel as the fiber is disposed in the ingot relative to the longitudinal axis of the ingot.

A still further object of the invention is to provide an improved method of forming wheels in which the number of necessary operations is reduced and the expense of making the wheels is materially lessened and by which wheels of an improved and superior quality are obtained.

The invention consists in an improved method of making wheels, comprising casting a multiple length blank, severing the cast blank transversely into wheel blanks and the succeeding forging operations by a series of novel steps by which wheels are produced in which the grain or fiber of the metal does not extend across the diameter of the wheels nor in a direction parallel with the axis of the cast blank but in the hub, 80 web and flanged portions is caused to extend in the same general direction axially outward at all points of the said portions.

The invention also consists in forming a metal blank with its axial central portion 85 formed from the axial central portion of the cast blank and then displacing metal from the cut face of the blank intermediate of the hub and periphery of the blank into the flange of the wheel.

The invention further consists in making forged metal wheels having a tread portion whose outer side or edge portion is formed of metal displaced from the periphery or marginal edge of the cast blank or ingot.

The invention still further consists in severing a blank transversely into wheel blanks and forging the severed blanks into wheels in such manner that the wearing surfaces of the tread and flange portion of the 100 finished wheels are formed from the cut surfaces of the severed blanks.

In the drawings, 2 represents a multiple length ingot or cast blank of circular or polygonal cross-section and 3 is the ingot after having been reduced transversely in area by rolling or forging. This reducing step is preferably employed, although it may be omitted within the scope of my broader claims and the single blanks may 110 be formed by transversely severing the cast ingot.

The ingot or multiple length blank is severed transversely by shearing, sawing, or in any other desired manner into wheel blanks 4 of the desired weight and thickness, the cut blank preferably being made at least as thick as the thickness through the hub of the finished wheel. The cut wheel blanks are re-heated and are then forged into finished wheels by means of suitable forming dies, either reciprocating dies, as shown in Figs. 4 to 8, rotary forging dies, or rocking forging dies similar to those shown in Figs. 9 to 11, having their axes at an angle to each other, being employed 15 to carry out the forging operation.

In carrying out the forging operation by means of the reciprocating dies shown in Figs. 4 to 8, the cut blank A is placed between the dies 5 and 6 of Fig. 4 in the position shown in full lines therein. The dies 5 and 6 are then caused to approach each other until the blank A is forged into the shape shown in cross-section between the dies 5 and 6 in Fig. 5. The partly formed 20 blank A is then removed to a second set of reciprocating forging dies 7 and 8, as shown in Fig. 6 and these dies are caused to approach each other until in the relative position shown in Fig. 7, so as to bend or dish the periphery of the blank A as is shown in cross-section between the dies 7 and 8 in Fig. 7. It will be noted that in the forging 25 operation in the first set of dies 4 and 5 the blank is decreased in thickness and is increased in diameter, a well defined hub portion being formed in this forging operation. In the second step of the forging 30 operation, as shown in Figs. 6 and 7, the blank is curved or bent into the dished form shown and the peripheral surface of the blank A in Fig. 4 is displaced so as to 35 form the outer edge of the one side of the dished blank shown in Fig. 7. The dished blank is then removed to a third set of reciprocating dies 9 and 10 where it is further reduced and in which the flange and tread portions are further developed and the blank is finished to size, as shown in Fig. 40 45 50 55 60 65 8. In the dies 9 and 10, the forging of the flange is completed and the flange is formed of metal displaced from between the marginal edge of the blank and its axial center, with the wearing surfaces of the flange and tread portions formed of metal originally 70 75 80 85 90 95 100 105 110 115 120 125 130 in the cut face of the blank A between its axial center and periphery.

In carrying out my improved method of forging the blanks by means of rotary or rocking dies having their axes at an angle to each other as shown in Figs. 9, 10 and 11, the blank A (shown in full lines) is placed between the dies 11 and 12 and the dies are caused to approach each other while rotating so as to form the metal into the shape 65 shown in dotted lines in Fig. 9. The partly

formed blank is preferably then removed to a second set of rotary forging dies 13 and 14 in which the blank is further reduced, the flange further developed and the wheel is forged from the shape shown in section in Fig. 10 into the finished shape as shown in Fig. 11.

In forging the blanks by means of the rotary or rocking dies having their axes at an angle to each other, the metal is displaced in a similar manner to that in the reciprocating forging dies and the entire wearing surface of the flange and tread portions is formed of metal originally in the cut face of the severed blank while the flange is entirely formed of metal displaced from between the axial center and the periphery of the blank, the flow of the metal in the periphery of the blank being indicated by the arrows.

While I have shown two sets of reciprocating dies and two sets of rotary or rocking dies having their axes at an angle to each other in carrying out the steps of forming a wheel, the number of sets of dies used may be increased or decreased, depending upon the amount of work necessary to reduce the blank to the finished article.

The advantages of my invention will be appreciated by those skilled in the art. By my improved method of forming the ingot, 95 severing the ingot into blanks and finally forging the blanks into wheels, as described, I am enabled to produce forged metal wheels having a fiber structure in which the grain or fiber does not cross the periphery of the finished wheel at any point and in which the grain or fiber of the finished wheel extends in the same direction relative to its axis at all points on its periphery.

The forging of wheels by my improved 105 method enables the forming of wheels having integral flange and tread portions in which the wearing surfaces of the flange and tread are formed from the cut surface of the blanks, the flange and tread portions 110 of metal located between the center and periphery of the blank in the sheared or cut surface of the severed blanks and in which the metal in the periphery of the cut blanks is displaced to the annular outer edge of the 115 tread portion of the wheel.

The wheel blanks may be punched either at the beginning of the forging operation or after the forging operation has been completed or the blank may be punched during an intermediate stage of the forging operation or simultaneously with the forging operation as is desired.

Modifications in the arrangement and construction of the dies may be made without departing from my invention. The ingot may be cast with a cylindrical or polygonal cross-section and may be of any desired length. The cross sectional area of the ingot may or may not be reduced prior to the shear-

ing operation; the manner in which the ingot is reduced in cross-sectional area and is severed into blanks may be changed; the number of forging steps carried out in forming the wheels may be varied; the weight and thickness of the blanks may be increased or decreased, and other changes may be made within the scope of the claims.

I claim.

10 1. The method of forming wheels, consisting in taking an ingot, severing transversely therefrom a blank having its axis extending in the same direction relative to the metal of the blank as the axis of the ingot extends 15 relative to the same metal, and then forcing metal intermediate the periphery and axial center outwardly to form the flange portion of the wheel; substantially as described.

2. The method of forming wheels, consisting in taking an ingot, severing transversely therefrom a blank having its axis extending in the same direction relative to the metal of the blank as the axis of the ingot extended relative to the same metal, and 25 then forcing metal intermediate the periphery and axial center outwardly to form the rim portion of the wheel; substantially as described.

3. The method of forming wheels, consisting in taking an ingot, severing transversely therefrom a blank having its axis extending in the same direction relative to the metal of the blank as the axis of the ingot extended relative to the same metal, and 35 then forcing metal intermediate the periphery and axial center outwardly to form the tread of the wheel; substantially as described.

4. The method of forming car wheels, 40 consisting in taking an ingot, severing transversely therefrom a blank having its axis extending in the same direction relative to the metal of the blank as the axis of the ingot extended relative to the same metal, and 45 then displacing metal intermediate the periphery and axial center outwardly to form the flange and tread of the wheel; substantially as described.

5. The method of forming wheels consisting in taking an ingot, reducing its cross-sectional area, severing transversely therefrom a blank having its axis extending in the same direction relative to the metal of the blank as the axis of the ingot extended 55 relative to the same metal, and then forcing metal located intermediate the periphery and axial center outwardly into the rim portion of the wheel and forming the wearing surface of the rim portion of the wheel of metal in the cut surface of the blank; substantially as described.

6. The method of forming wheels, consisting in taking an ingot severing transversely therefrom a blank having its axis extending 60 in the same direction relative to the metal of

the blank as the axis of the ingot extended relative to the same metal, and then forcing metal intermediate the periphery and axial center outwardly in the rim portion of the wheel and forming the periphery of the 70 wheel of metal in the cut face of the severed blank; substantially as described.

7. The method of forming wheels, consisting in taking an ingot, reducing its cross-sectional area, severing transversely 75 therefrom a blank having its axis extending in the same direction relative to the metal of the blank as the axis of the ingot extended relative to the same metal, and then forcing metal intermediate the periphery and 80 axial center outwardly into the flange of the wheel and forming the wearing surface of the wheel flange of metal from the cut face of the severed blank; substantially as described.

8. The method of forming wheels, consisting in taking an ingot, severing transversely therefrom a blank having its axis extending in the same direction relative to the metal of the blank as the axis of the ingot extended 90 relative to the same metal, and then forcing metal intermediate the periphery and axial center outwardly into the flange of the wheel and forming the wearing surfaces of the flange and tread portions of the wheel of 95 metal displaced from the cut face of the severed blank; substantially as described.

9. The method of forming wheels, consisting in taking an ingot, severing transversely therefrom a blank, forging the blank into a 100 wheel and displacing metal to form the wearing surfaces of the flange and tread portions of the wheel from metal in the cut face of the severed blank; substantially as described.

10. The method of forming wheels, consisting in taking an ingot, reducing the cross sectional area of the ingot, severing transversely therefrom a blank having its axis extending in the same direction relative to the metal of the blank as the axis of the ingot extending relative to the same metal, and 110 then forcing metal intermediate its periphery and axial center outwardly to form the flange portion of the wheel; substantially 115 as described.

11. The method of forming wheels, consisting in taking an ingot, reducing the cross sectional area of the ingot, severing transversely therefrom a blank having its axis 120 extending in the same direction relative to the metal of the blank as the axis of the ingot extended relative to the same metal, and then forcing metal intermediate its periphery and axial center outwardly to form the 125 rim portion of the wheel; substantially as described.

12. The method of forming wheels, consisting in taking an ingot, reducing the cross sectional area of the ingot, severing 130

transversely therefrom a blank having its axis extending in the same direction relative to the metal of the blank as the axis of the ingot extended relative to the same metal, and then forcing metal intermediate its periphery and axial center outwardly to form the tread of the wheel; substantially as described.

13. The method of forming car wheels, 10 consisting in taking an ingot, reducing the cross sectional area of the ingot, severing transversely therefrom a blank having its axis extending in the same direction rela-

tive to the metal of the blank as the axis of the ingot extended relative to the same metal, and then displacing metal intermediate its periphery and axial center outwardly to form the flange and tread of the wheel; substantially as described.

In testimony whereof, I have hereunto set 20 my hand.

EDWIN E. SLICK.

Witnesses:

R. D. LITTLE,  
H. M. CORWIN.